

Oct. 8, 1935.

C. S. DIPPEL

2,016,416

METHOD OF MAKING A PATTERN RECORD

Filed Sept. 4, 1931

FIG. 1.



FIG. 2.



FIG. 3.



INVENTOR  
C. S. DIPPEL

BY  
E. R. Nowlan

ATTORNEY

## UNITED STATES PATENT OFFICE

2,016,416

## METHOD OF MAKING A PATTERN RECORD

Cornelius S. Dippel, Woodcliff, N. J., assignor to  
Western Electric Company, Incorporated, New  
York, N. Y., a corporation of New York

Application September 4, 1931, Serial No. 561,142

8 Claims. (CL. 41—41)

This invention relates to patterns and to a method of reproducing them, and more particularly to a method of transferring to any desired surface a facsimile or image of the grain of wood.

5 It frequently becomes desirable to produce new articles of relatively cheap wood such as pine, bass, gum, birch, or of metal, or to refinish articles that have become scratched or marred in service so that they shall have a finished appearance closely approximating that of a rare or expensive wood, such as walnut or mahogany. To accomplish this, several methods have been employed at various times in the past in preparing a surface containing a grain pattern which 10 is to be reproduced. These methods have in some instances involved an etching away of portions of the wood, such as by treatment with an acid or a caustic solution, or a solvent capable of dissolving portions of the wood, or by charging. 15 In other instances, the selected grain pattern has been photographed, and an etching has been made on a copper plate from the photograph. It has also been the custom, in some instances, to entirely cover the surface on which the grain 20 pattern was to be reproduced, with a flat ground coat of paint that, in the case of its application to wood, completely blotted out the surface characteristics and grain pattern.

25 Objects of the present invention are to prepare and reproduce wood and other grain patterns, as well as the surface characteristics of other substances, the method of reproducing being applicable to any smooth surface, and resulting in faithful reproduction of details and very close 30 resemblance to natural finish.

35 In the preferred embodiment of the invention, a smoothly machined surface of wood containing a selected grain pattern is treated with a non-corrosive salt solution by vigorous brushing, which removes foreign matter from the pores of the wood. It is then coated with an organic protective coating, after which it is inked and an impression of the grain pattern is transferred by means of a roll to a stained wood surface.

40 45 Other features and advantages of the invention will become apparent from the following detailed description of one embodiment thereof, reference being had to the accompanying drawing wherein

50 Fig. 1 is a plan view of a surface of a piece of wood containing a grain pattern that is to be reproduced;

55 Fig. 2 is a plan view of a similar surface, showing an inked impression of the grain pattern partially transferred to a roll, and

Fig. 3 is a plan view of a surface upon which a grain pattern is to be reproduced, showing the inked impression of the grain pattern partially deposited thereon by the roll.

Referring now to Figs. 1 and 2 in the drawing in which like numerals designate like parts throughout the several views, 10 is a selected piece of wood having a surface 11 containing a grain pattern 12 which it is desired to reproduce on another surface. In Fig. 2, the reference numeral 14 indicates a portion of the surface 11 which has been treated with ink, pigment, or paint. A printer's roll or gelatine or other transfer roll is indicated at 15, and it has been rolled partially across the surface 11, as a result of which an impression 16 of the grain pattern has been transferred to that portion of the roll 15 that has been in contact with the surface 11. When the roll 15 has received the complete impression of the surface of the piece of wood 10, the impression may be transferred to any desired smooth surface.

In Fig. 3, the reference numeral 18 designates a portion of any smooth surface, on which the grain pattern is to be reproduced. The roll 15 is shown with the impression 16 of the grain pattern completely transferred thereto. The roll 15 has been drawn partially across the surface 18, and has impressed thereon a reproduction 19 of the grain pattern.

30 35 In preparing the surface 11 in accordance with the preferred form of the invention, it is first carefully dried and then machined in any suitable manner so as to be as level and smooth as possible. The surface is then polished with suitable fine abrasives, such as pumice stone. The polishing is done with any suitable volatile vehicle for the abrasive, such as benzene, toluene, turpentine, etc. The polishing vehicle must be a substance that will not affect the subsequent 40 coats of finishing material.

45 After the surface has been sufficiently polished, it is permitted to dry thoroughly. It is then treated with a water solution of a non-corrosive salt. Alum, chemically known as sodium tetraborate and borax, chemically known as potassium-aluminum sulphate, have been found to give particularly satisfactory results, although other water solutions of salts which dissociate electrolytically in water may be used, providing their 50 water solutions are non-corrosive. The term "non-corrosive" as used herein in connection with salts and their aqueous solutions, is to be interpreted as signifying that no portions of the wood are softened, jellified, or dissolved by the 55

action of the salt or the solution. In the preferred embodiment of the invention, a saturated solution is employed, but the invention is not to be construed as limited to the use of a saturated solution, as comparatively satisfactory results may be obtained by using dilute solutions, and to a lesser degree by using clear water. A short, fine, stiff-bristled brush is dipped in the salt solution and the solution is applied to the grained surface by a vigorous brushing parallel to the grain. The brushing is continued until all foreign matter is removed from the pores and the surface of the wood. It is possible to remove foreign matter from the pores of the wood by dry brushing with a fine, stiff-bristled brush, such as a brush having bristles of fine brass wire. However, it has been found more satisfactory to use a solution in connection with the brushing.

When the wood has completely dried, the surface is lightly sanded, and all dust is removed. The surface is then covered with any suitable organic protective coating, such as nitrocellulose lacquer or other lacquer, which serves several purposes. It preserves the surface of the wood and protects the raised fibres, it stops the absorptive nature of the wood and makes it impervious to transfer fluids such as ink, paint or pigment, and it produces a smooth hard surface from which an impression may conveniently be taken. After the lacquer has completely dried, the wood is sanded lightly until the surface is smooth. If the surface is not sufficiently smooth one or more additional coats of organic coating may be applied, until a satisfactory surface is obtained.

The next step in the process is to completely cover the smooth lacquered surface with suitable transfer fluid ink, paint, or pigment, and to wipe away the excess, leaving the pores of the wood filled with and the surface substantially free from the fluid. A roll of the type commonly referred to as a printer's roll, or a soft transfer roll, is rolled across the inked or painted surface that contains the grain pattern. The soft surface of the roll contacts with the inked or painted pores of the wood and receives therefrom a faithful reproduction of the grain pattern. The grain pattern is then ready to be transferred to the desired surface. This may be accomplished by the simple operation of rolling the inked roll across the surface. A reproduction, in ink, of the wood grain pattern will be deposited on the surface. After the ink has dried, finishing coats of suitable organic substances may be applied over the reproduced grain pattern.

When the grain pattern is to be reproduced on wood, the most satisfactory results can be obtained by choosing wood that has an even texture, and a fine, close, straight grain, substantially free from prominent or distinctive patterns. Pine, birch, bass, gum, etc., are examples of wood especially suited to receive artificial grain patterns. The wood is machined to the desired smoothness by any suitable method, after which it is stained. The color of the stain used is dependent upon the finish that is to be applied, an example of this being the use of walnut, oak, or mahogany stain, for corresponding grain patterns. The stain serves as an undertone and gives color to the surface of the wood without destroying its identity as wood.

The natural grain pattern of the wood is not blotted out, but its prominence is reduced, and

uniformity of surface is obtained. The fact that the grain of the wood shows through the stain makes apparent the desirability of using fine grained wood, as mentioned above. The stained surface serves as a background for the artificial grain pattern, enables the finished surface to retain a natural wood appearance, and gives to the grain pattern impressed thereon an appearance of naturalness and depth, so that the surface is very definitely identified as a wooden and not a metal or other surface.

The process of reproducing patterns hereinbefore described is capable of wide application. It may be used to reproduce characteristic features of wooden surfaces, such as grain, feather, 15 burls, knots, or of other surfaces such as leather, fibre, textiles, paper, etc., on surfaces of wood, metal, glass, ceramic materials, fibre, leather, paper, fabrics, rubber, etc. It is to be understood that the method of the present invention is not 20 limited to the specific application herein illustrated and described, but is capable of numerous applications within the scope of the appended claims.

What is claimed is:

1. A method of preparing a wooden surface for use as a master record in reproducing a wood grain which comprises treating the surface with a non-corrosive water solution of an electrolytically dissociable salt to accentuate the grain pattern.

2. A method of preparing a wooden surface for use as a master record in reproducing a wood grain which comprises brushing the surface with an alum solution to remove foreign materials and to accentuate the grain pattern, and covering the surface with a protective coating.

3. A method of preparing a wooden surface for use as a master record in reproducing a wood grain which comprises treating the surface with a borax solution to remove foreign materials and to accentuate the grain pattern, and covering the surface with a protective coating to make it impervious to transfer fluid.

4. A method of preparing a wooden surface for use as a master record in reproducing a wood grain which comprises treating the surface with an alum solution to remove foreign materials and to accentuate the grain pattern, and covering the surface with a coating of lacquer.

5. A method of preparing a surface for use as a master record in reproducing surface characteristics, which comprises treating the surface with an alum solution to accentuate the surface characteristics.

6. A method of preparing a wooden surface which comprises treating the surface with an alum solution to remove resins and foreign materials, and to accentuate the grain pattern, and covering the surface with a protective coating.

7. A method of preparing a wooden surface for use as a master record in reproducing a wood grain which comprises the steps of treating the surface with a non-corrosive water solution of an electrolytically dissociable salt, and subsequently applying a protective coating to the surface.

8. A method of preparing a wooden surface for use as a master record in reproducing a wood grain which comprises the steps of treating the surface with a non-corrosive water solution of an electrolytically dissociable salt, and subsequently applying a permanent coating to the surface.